

## UNITED STATES PATENT OFFICE

2,287,771

## PRODUCTION OF POWDERED ALLOYS

Peter P. Alexander, Marblehead, Mass.

No Drawing. Application January 9, 1940,  
Serial No. 313,116

6 Claims. (Cl. 75—0.5)

This invention relates to the production of powdered alloys, and more especially to the production of finely divided powdered alloys of the refractory and other metals with one another or with carbon, iron, nickel and cobalt.

The formation of alloys of the refractory metals, is, in general, well known and may be brought about, for example, in the electric furnace. However, the production of alloys of these metals in the form of finely divided powders capable of passing, say 200 mesh or better, is attended with considerable difficulty. Generally speaking, the alloys are extremely hard and, when produced according to any known or previously used process, take the form at best of large particles which must be ground to produce the degree of fineness necessary for many industrial purposes, a difficult operation. If the metals in the form of fine powders are simply fused together they form large particles or even blocks of extreme hardness, the difficulty of reducing the latter to fine powders being even greater.

According to the present invention, powdered alloys of the metals fine enough to pass 200 mesh or better are produced without the necessity of subjecting the same to crushing or grinding operations.

The process of the invention does not depend, for fineness in size of the powdered alloys produced thereby, upon the degree of preliminary crushing and grinding of the metals entering into the alloys. While the process is carried out with powdered and thoroughly mixed materials, nevertheless the particles of the final alloy are much smaller and more uniform in size than those of the initial powdered materials. This is brought about in the process by the decomposition of the initial mixture which, in the preferred form is accomplished partly by the introduction of one of the metals, into the initial mixture, in the form of an oxide, which is reduced at a temperature below the fusion temperature of the metal, and partly through the formation, during the early heating stages of the process, of complex compounds of the other metal which are reduced or otherwise broken up at low temperatures below the point of fusion of either alloying metal.

In order that the fine particles of metal may unite to form fine particles of alloy, the process is further characterized by the fact that it is carried out under conditions wherein the atmosphere is highly reducing and free from oxygen, thus preventing surface oxidation of the particles of the metals which, being free from oxide, may weld and diffuse into one another. Moreover, the process is characterized by the fact that there is brought about, during one phase thereof, a certain amount of movement of the metallic particles towards one another which is accompanied by the formation of a spongy spacer which will

permit only the welding and diffusion of adjacent particles and prevent the coagulation and sintering of the particles of the alloy or its constituents into larger masses.

5 The various phases of the process are carried out in a relatively simple manner as follows:

The powdered oxide, for example, of one of the refractory metals which is to form a part of the alloy, is thoroughly mixed with the alloying metal in powdered form. A powdered metal hydride, for example calcium hydride, is added to the mixture in sufficient amount to carry out the reactions hereinafter described, the whole being thoroughly mixed so that the particles of the powdered metal hydride are scattered through the mass of powdered metal and oxide. The powdered charge is placed in a furnace and the temperature raised until the metal hydride dissociates forming nascent hydrogen and the metal released from the hydride, the latter being in a nascent state. Inasmuch as the density of calcium hydride is 1.7 and that of metallic calcium 1.55, it will be apparent that after dissociation the released calcium occupies a larger volume than the calcium hydride. There will therefore be an expansion of every particle which previously was composed of calcium hydride, this expansion pushing the adjacent particles of metallic oxide and metal together. At the same time the large volume of evolving hydrogen in the mass produces a further movement of the particles towards one another. As the hydrogen evolves in the mass it also reduces the metallic oxide to particles of metal and oxygen, the latter uniting with the hydrogen to form steam which is immediately reduced by the calcium, the latter uniting with the oxygen to form calcium oxide while the hydrogen escapes.

40 The density of the calcium oxide is much greater than that of the calcium so that there is now a contraction of the particles which were originally calcium hydride, the calcium oxide forming a spongy mass comprising countless elemental crucibles surrounding the particles of the metals which, during the continued application of heat are welded together and diffuse into one another, the presence of the highly reducing hydrogen in the mass preventing the formation of surface oxides on the metallic particles so that the welding and diffusion may take place. Sintering of adjacent particles of alloy into a spongy mass or into larger particles is prevented by the surrounding calcium oxide.

45 As a further aid to the understanding of the invention I will now describe the formation of a specific powdered alloy made in accordance with the invention, in this instance titanium carbide.

50 Powdered calcium hydride and powdered titanium oxide are thoroughly mixed with powdered carbon, preferably in the form of "lamp black."

The temperature of the charge is raised to 960° C. to 1000° C. The reaction starts at about 700° C., the calcium hydride dissociating to form nascent calcium and nascent hydrogen, the latter reducing the titanium oxide to form particles of metallic titanium and oxygen, the hydrogen combining with the latter to form steam. The steam is immediately reduced by the calcium to form calcium oxide and hydrogen, the hydrogen being permitted to escape. As the temperature increases the adjacent particles of titanium and carbon in each elemental crucible are welded together, the application of heat being continued until the particles of welding titanium and carbon diffuse into one another forming finely divided particles of titanium carbide. The reaction may be expressed as follows:



When the reaction is complete the calcium oxide may be removed in any well known manner, for example, by leaching, leaving powdered titanium carbide.

As far as I am now aware the process is more or less limited to the use of calcium, strontium and barium hydrides as reducing-spacer-forming agents as other reducing agents, such as aluminum, will readily combine with one or more of the metals to be alloyed and furthermore the heat of reaction during the first stage would be so great that the whole mass would be fused. In the case of calcium, strontium and barium hydrides the heat of reaction is very much lower so that the whole process is carried out below the point of fusion and therefore the material comes in fine solid particles of alloy. It is possible that other reducing spacer-forming agents may be substituted for those enumerated but in commercial operation I prefer to use calcium hydride as the other agents have no marked advantage over calcium hydride whereas the latter is much cheaper commercially than barium or strontium hydrides. Moreover calcium hydride may be prepared according to the method disclosed and claimed in my prior Patent No. 2,082,134, issued June 1, 1937, it being immaterial, insofar as the present method is concerned, whether or not all traces of magnesium oxide are removed.

There are further apparent limitations of the process, namely, that the alloying metals must combine more readily with one another than with the metal liberated from the reducing-spacer-forming agent, thus, while the metals, titanium, zirconium, tungsten, hafnium, thorium, tantalum, uranium, molybdenum, chromium and beryllium may be alloyed with one another or with carbon, nickel, iron and cobalt, in accordance with the process, they may not be alloyed with silicon, copper and magnesium, which combine and form stable compounds with calcium.

During the early heating stages, before the calcium hydride is reduced to calcium and hydrogen, it is probable that the powdered metal forms complex compounds with the calcium hydride, these compounds breaking up as the temperature increases. I do not commit myself as to the nature of these compounds. Suffice it to say that the formation of such compounds accounts partly for the fact that the size of the particles of the final alloy is, in general, much smaller and more uniform than the powdered oxide and powdered metal of the initial mixture.

It will be understood by those skilled in the art that the length of time that the heat treatment

must be continued to effect diffusion of the particles into one another will vary in accordance with the metals of the group which are selected to form the alloy.

While I have described my process with great particularity, it will be understood that the same may be varied within the spirit of the invention and the scope of the appended claims.

What I claim is:

10. The process of forming powdered alloys consisting of a metal selected from a first group consisting of titanium, zirconium, tungsten, hafnium, thorium, tantalum, uranium, molybdenum, chromium and beryllium and an alloying element selected from a second group consisting of titanium, zirconium, tungsten, hafnium, thorium, tantalum, uranium, molybdenum, chromium, beryllium, carbon, nickel, iron and cobalt which comprises thoroughly mixing a powdered oxide of the metal of the first group with powdered calcium hydride and the alloying element of the second group in powdered form, raising the temperature of the mixture to the point where the hydrogen is liberated from the calcium hydride, the liberated hydrogen reducing the metal oxide whereupon the calcium combines with the oxygen to form calcium oxide, and thereafter further raising the temperature to the point where the metal liberated from the oxide diffuses into the alloying element from the second group.
20. The process of forming powdered alloys consisting of a metal selected from a first group consisting of titanium, zirconium, tungsten, hafnium, thorium, tantalum, uranium, molybdenum, chromium, beryllium, carbon, nickel, iron and cobalt which comprises thoroughly mixing a powdered oxide of the metal of the first group with the alloying element in powdered form and a powdered metal hydride selected from a group consisting of calcium hydride, barium hydride and strontium hydride, raising the temperature of the mixture to the point where the hydrogen is liberated from the metal hydride, the liberated hydrogen reducing the metal oxide whereupon the oxygen liberated therefrom combines with the metal liberated from the metal hydride, and thereafter further raising the temperature until the metal of the first group diffuses into the alloying element of the second group.
30. The process according to claim 1 in which the amounts of powdered oxide and alloying elements are varied in accordance with the desired percentages in the final alloy whereas the amount of calcium hydride is varied in accordance with the amount of the metal oxide present.
40. The process according to claim 2 in which the amounts of metal oxide and alloying elements are varied in accordance with the desired percentages in the final mixture whereas the amount of metal hydride is varied in accordance with the amount of the metal oxide present.
50. The process according to claim 1 in which after diffusion of the metal into the alloying element the calcium oxide is removed by leaching the same.
60. The process according to claim 2 in which after diffusion of the metal into the alloying element the metal oxide formed by the metal hydride is removed by leaching the same.

PETER P. ALEXANDER.